

May 30, 1933.

D. FINLEY

1,911,357

COVERING MATERIAL AND METHOD OF MAKING THE SAME

Filed May 24, 1927

Fig. 1



Fig. 2



INVENTOR  
DOZIER FINLEY

BY *Charles S. Evans*  
HIS ATTORNEY.

## UNITED STATES PATENT OFFICE

DOZIER FINLEY, OF BERKELEY, CALIFORNIA, ASSIGNOR TO THE PARAFFINE COMPANIES, INC., OF SAN FRANCISCO, CALIFORNIA, A CORPORATION OF DELAWARE

## COVERING MATERIAL AND METHOD OF MAKING THE SAME

Application filed May 24, 1927. Serial No. 193,928.

My invention relates to a method of applying a wearing coat to the surface of a base in the manufacture of floor and wall coverings.

5 One of the objects of my invention is the production of a covering in which a wider range of color effects can be secured than has been possible heretofore.

Another object of my invention is the production of a covering in which the entire surface, or selected areas thereof, are coated with a light reflecting substance to enhance the brilliancy and depth of the coloring.

Another object of my invention is the production of a covering, the entire surface or portions of which are coated with a transparent material.

My invention possesses other objects and valuable features, some of which will be set forth in the following description of my invention which is illustrated in the drawing forming part of the specification. It is to be understood that I do not limit myself to the showing made by the said description and drawing, as I may adopt varying forms of my invention within the scope of the claims.

Figure 1 is a vertical sectional view of my covering material showing the transparent and opaque portions of the coating.

Figure 2 is a vertical sectional view showing the application of a light reflecting medium disposed under the transparent portion of the coating.

35 Floor coverings of the type known as felt base floor coverings have been made according to a practically unvarying procedure since the beginning of the industry. Briefly this procedure comprises saturating a 40 base sheet, preferably felt, with an asphaltic compound having a melting point of from 115° F. to 145° F. This saturated sheet is then coated on both sides with linseed oil or China-wood oil base paint, the underside, 45 which is designed to lie next to the floor, receiving a comparatively thin coating in which sufficient pigment is carried to hide the black color of the base. The upper surface receives a much thicker coating which 50 may be designated as a "seal coat" as it

seals the asphalt in the base and prevents its black color from bleeding thru into the print coats which are superimposed upon the seal coat. The print coat is practically a pigmented varnish enamel which is applied by means of a system of block printing. The print coat, when dried, constitutes the final finish of the floor covering. The surface is enamel-like in character due to the fact that varnish has been used in the 60 print paint. The enamel-like surface thus produced is usually deemed sufficient for a final finish, but there are certain manufacturers who are making such printed floor coverings and applying over the printed surface a finish surface coating comprising a nitrocellulose lacquer. It has not been uncommon to apply varnish over the surface of printed floor coverings either before or after they have been put into service. The 70 present invention does not, however, have anything to do with the practice of merely varnishing or lacquering the surface.

Before taking up the various steps of the process, it is necessary that consideration be given the matter of light absorption and reflection. In the manufacture of floor coverings as just explained, the enamel paint composing the printed surface provides but one method of producing color effects. The 80 paint is composed of a more or less light colored oil and varnish mixture and has ground into it pigments of such character as zinc oxide, with or without tinting colors such as ultra-marine blue. No matter what may be the character of the pigment, the color is seen by the observer in accordance with the following phenomena. Light from the prevailing source is directed to the surface of the floor covering where it passes thru an almost infinitely thin layer of oil varnish and strikes the uppermost layer of pigment particles. If there is no preferential absorption of the various component colors in the original white light, then practically all of the white light is again diffused outwardly and the observer sees a white area on the surface of the covering. If on the other hand, there is an absorption 90 of practically all of the components of the 95 100

white light except the green, this green is diffused outwardly and the observer sees a green area. It will thus be observed that the light absorption has taken place at the surface of a solid particle of matter and has not been brought about by the absorption of component colors of the white light while the light was traveling thru an appreciable thickness of transparent material.

10 There is another type of light absorption of which no advantage has ever been taken in the printing of floor coverings. This type of light absorption is obtained when the light is passed thru a colored glass or a 15 colored medium of any description which has the characteristics of transparency or translucency. It is a type of absorption which is entirely different from that which takes place when light hits an opaque object 20 and is again thrown away from that object. The fact that white or any other colored light from an opaque surface appears different from the same color of light which is passed thru a transparent colored medium 25 is a matter of common experience. It is with the object of taking advantage of this fact that the present invention has been developed.

Broadly, my invention relates to the method 30 of applying a wearing surface to a base, which comprises first overlaying all or selected areas of the surface with a light reflecting material over which a transparent wearing or service coating is applied. The 35 transparent coating is preferably applied only over the surface which has previously been overlaid with the light reflecting material. When only selected areas are covered in this manner, the remaining areas are 40 preferably covered with the usual paint coats. If desired the transparent coating may be colored by suitable dyes or stains or color effects can be secured by using a colored light reflecting medium.

45 In detail, the method of my invention is carried out as follows: A base 2, preferably a felt sheet such as is customarily used in the manufacture of floor covering, is treated with a linseed oil or a China-wood oil 50 base paint and covered with the usual "seal" coat 3. The base is then ready to receive the wearing or service coat and up to this point my method is the same as that previously employed. In carrying out my 55 process, it is preferable that certain areas be selected on which the method of printing of this invention will be applied. For example, it will be found particularly applicable to the petals and leaves of flowers, but 60 is of course not necessarily confined to this use, as the entire surface may be so coated if desired.

When selected areas are to be covered in accordance with this method, such selected 65 areas are first coated with a light reflecting

material 4, preferably a bronzing liquid composed of polished flake aluminum powder mixed with any suitable vehicle such as shellac or spar varnish thinned with benzole. If desired, a clear dye or stain may be 70 incorporated in the light reflecting coating to give a colored background. The design is then printed on the floor covering using the printing blocks in the normal manner with the exception that a varnish is used 75 on the printing blocks for the selected areas, while the usual print paint is used on the blocks printing the remaining areas. In other words a surface is provided in which selected areas are overlaid with a trans- 80 parent coating 6 while the remaining areas are covered with an opaque coating 7. In order to produce a smooth surface it is essential that the thickness of both the print coat and the varnish coat be the same. It 85 will thus be obvious that a transparent coating of varnish, having an appreciable thickness is provided, and since the light absorption in a transparent coating is so different from that in an opaque surface, these areas 90 are emphasized so that very attractive contrasts can be secured.

The varnish coating may, if desired, contain an oil soluble stain. For example, if the petals of a red rose are to be represented, the varnish probably would be stained with a soluble red dye and if the leaves were to be represented, a soluble green dye would be dissolved in the varnish. When adding these stains, consideration 95 must be given to the thickness of the coat. A thin transparent object appears to have a much lighter color than a thick one, and since the transparent varnish coat is of appreciable thickness, care must be taken to 100 secure the color desired.

When the surface of the floor covering is dry, the areas covered with the transparent coating appear to lie in different planes than the areas covered with the opaque coating. There is also a difference in the character of the colors produced in the two types of coatings so that a wide range of 110 color combinations and effects can be secured.

Very satisfactory results have also been obtained by the use of a metal foil 8 in place of the light reflecting paint. Such a foil is preferably cemented onto the base 115 and may be the natural color of the metal or it may be colored. Pleasing effects have been produced by allowing the foil to wrinkle slightly while being secured to the base. The transparent varnish coating 9 is applied over the foil in the same manner as when a light reflecting metallic paint is used. When the light reflecting surface is colored, a clear varnish may be used if desired, or varnishes of contrasting colors may 125 130 135 140 145 150 155 160 165 170 175 180

be employed to produce very unusual effects.

I have referred to the use of a transparent varnish coat throughout the specification, and while spar varnish is probably the best suited for this use, there are other coating materials which may be employed. For example, the following may be used in place of spar varnish: flooring or furniture varnishes, lacquers, preferably the lacquers having a base of cellulose esters, and some of the phenol condensation products commonly referred to as synthetic resins. I have explained my process as applied to floor coverings which are made in a printing machine, but it is obvious that the same results can be obtained by the application of the varnish with a brush or spray.

I claim:

20 1. The process of applying a service coating to a base which comprises applying on selected areas of the base a vehicle containing light reflecting material and a dye to provide a colored light reflecting film, covering only said selected areas of the base with a transparent coat, and covering the remaining surface of the base with an opaque coat, whereby the transparent coated areas are emphasized and made to appear to lie in a different plane from the opaque coating.

25 2. An article of manufacture comprising a base, a light reflecting film on a selected area of said base and comprising light reflecting material and dye held in a vehicle which adheres to the base, a transparent coat disposed only over said film, and an opaque coating on said base and adjacent said transparent coat, whereby the transparent coated area is emphasized and made to appear to lie in a different plane from the opaque coating.

In testimony whereof, I have hereunto set my hand.

DOZIER FINLEY.